

Sept. 13, 1932.

W. R. GREIG

1,876,665

PIPE COVERING

Filed June 29, 1929

Fig. 1



Fig. 2



Fig. 3



INVENTOR  
WILLIAM R. GREIG  
BY  
Charles S. Evans  
HIS ATTORNEY

## UNITED STATES PATENT OFFICE

WILLIAM R. GREIG, OF BERKELEY, CALIFORNIA, ASSIGNOR TO THE PARAFFINE COMPANIES, INC., OF SAN FRANCISCO, CALIFORNIA, A CORPORATION OF DELAWARE

## PIPE COVERING

Application filed June 29, 1929. Serial No. 374,710.

My invention relates to coverings for protecting pipes from the corrosive action due to ground water with its dissolved salts, electrolysis, and the like.

5 The preferred material for such covering is fabric, such, for example, as a rag felt, which is saturated with water resistant material, usually of a bituminous character. The value of such coverings depends largely 10 upon complete continuity, but as the pipes are necessarily subjected to a certain amount of handling after the covering is applied, and as the fabric covering used is rather sensitive to abrasions, there is a likelihood 15 that the covering may be broken.

It is one of the objects of my invention, therefore, to provide a covering which will be highly resistant to abrasion.

Another object of my invention is to provide 20 a pipe covering which may be applied as readily as the ordinary abrasion sensitive type.

Yet another object of my invention is to provide a pipe covering having a light-reflecting surface, which will prevent the pipes, lying in the sun before being laid, from rising to a temperature so high as to make their handling difficult, and to cause running or oozing of the water resistant material.

30 Still another object of my invention is to provide an abrasion resistant pipe covering in which the abrasion resistant surface does not itself offer a point of ingress for the fluids which cause corrosion.

35 A further object of my invention is to provide a covering of the character described which is itself of moderate cost, and which may be applied with no greater expense than that involved in the use of coverings of the 40 ordinary type.

My invention possesses other objects and valuable features, some of which will be set forth in the following description of my invention which is illustrated in the drawing 45 forming part of the specification. It is to be understood that I do not limit myself to the showing made by the said description and drawing, as I may adopt varying forms of my invention within the scope of the claims.

50 Referring to the drawing:

Figure 1 depicts the covering of my invention as applied to a section of pipe.

Figure 2 is a view similar to Figure 1, and showing my invention in a modified form.

Figure 3 is a detailed sectional view showing the lap joint used in the preferred form of my invention.

Broadly considered, the pipe covering of my invention comprises a sheet or strip of fabric which is impregnated with a water 60 resistant material, and to the outer surface of which is cemented a sheet of abrasion resisting material, such as a tough, dense paper. The covering material is preferably formed in rolls, from which it may be applied spirally 65 to the pipe, either by hand or by a machine.

Describing a preferred embodiment of my invention in greater detail, the reference character 6 indicates a sheet of fabric which may be a woven material such as a cotton or 70 burlap sheeting, but is preferably a felted material such as is used as a base for sheet roofing. There is a wide choice of such materials, including asbestos and other mineral felts, but the so-called rag felt is low in price 75 and quite satisfactory for the purpose. The fabric sheet is impregnated or saturated with a water resistant material. The saturants may also be widely varied; asphalt, stearine pitch, coal or pine tar, and various gums and 80 oils, either alone or in combination, being suitable. The preferred material is an asphalt having a softening point of approximately 110° Fahrenheit, and a penetration of approximately 200 at 77° Fahrenheit, 100 85 grams, 5 seconds, by the methods of the American Society for Testing Materials, standards of 1927. If a woven fabric is used, the saturant should be harder, and should fill the interstices between the meshes 90 completely.

Secured to the fabric 6 by a layer of cement 7 is a sheet 8 of abrasion resistant material. A suitable cement is an asphalt which is harder than that used as the saturant, one 95 having a softening point of 180° F., and a penetration of 20 at 77° F., 100 grams, 5 seconds, A. S. T. M., standards of 1927, having been found satisfactory in practice. The cement is preferably applied to the felt as a 100

coating, the under side of the fabric being coated or uncoated, as may be preferred from manufacturing considerations.

5 A suitable abrasion resisting material is a tough kraft paper, which is preferably unsaturated and applied to the strip of fabric as a narrower strip, one edge of which coincides with that of the fabric, thus leaving a portion of the other edge exposed to form a 10 lap surface 9, as best shown in Figure 3.

Besides its abrasion resistant function, the paper, by virtue of its light-reflecting surface, serves to limit the temperature to which the 15 covered pipe will rise when stored in the sun, and so, not only make its handling easier, but also prevent running or oozing of the saturant.

The covering formed as described is preferably made into rolls, from which it may 20 conveniently be applied to the pipe.

This may be done either by hand or by machine. However the application is made, the pipe is preferably first prepared with a priming coat of asphaltic paint 12, covered by a 25 layer of cement 13. A satisfactory material for the latter is an asphalt with a softening point of 145° F., and a penetration between 30 and 40, at 77° F., 100 grams, 5 seconds, A. S. T. M., standards of 1927. This same material mixed with equal parts of gilsonite fused and cut with gasoline to a brushing consistency, may also be used for the priming 30 coat of paint.

35 The covering is wrapped spirally about the pipe, each turn of the coveringlapping over the exposed portion of the felt so that the entire outer surface of the pipe is covered with paper. Since the paper does not extend materially into the lap joint, there is 40 no tendency for it to conduct moisture by capillarity to a point where it could reach the pipe.

45 Where the pipe is to be used in conditions of unusual severity as to temperature, concentration of salt, or strong electric ground current, the protective coating may be applied over an inner wrapping of felt 14, as is shown in Figure 2. In this case, of course, 50 only the outer wrapping need be protected by the abrasion resisting covering.

55 Where the rise in temperature of the pipe, due to absorbed radiation, need not be considered, the paper coating may be saturated with a material of the same character as is used on the felt. In this case, both the paper and the felt may be of the same width, since the saturated paper will not conduct moisture. This construction is also shown in Figure 2.

60 Kraft paper, also known as "Swedish manila" or "express" paper, is the preferred material for the abrasion resistant layer, because of its tough, dense character and low cost. Other papers may, of course, be substituted, as, for example, sulphite papers.

I claim:

1. A pipe covering comprising a strip of fabric saturated with a water resistant material, and a strip of abrasion resistant material having a width less than the fabric strip and cemented thereto, one edge of said abrasion resistant strip spaced from an edge of the fabric strip to provide a lap surface. 70

2. A pipe covering comprising a strip of bitumenized fabric, and a strip of paper cemented thereto, one edge of said fabric strip being exposed to form a lap surface. 75

3. A protected pipe comprising a tubular member, and a wrapping on said pipe comprising a sheet of fabric saturated with a waterproof material and a sheet of abrasion resistant material cemented thereto so as to leave an edge of said fabric exposed, said wrapping being lapped to cover the exposed edge of the fabric. 80

In testimony whereof, I have hereunto set my hand.

WILLIAM R. GREIG.

90

95

100

105

110

115

120

125

130